

April 5, 1960

A. L. BREEN

2,931,091

CRIMPED TEXTILE FILAMENT

Filed Feb. 26, 1954

2 Sheets-Sheet 1

Fig. 1.



Fig. 4.



Fig. 2.



Fig. 5.



Fig. 3.



INVENTOR

Alvin L. Breen

BY C. H. Mortenson

ATTORNEY

April 5, 1960

**A. L. BREEN**

2,931,091

## CRIMPED TEXTILE FILAMENT

Filed Feb. 26, 1954

2 Sheets-Sheet 2



INVENTOR

INVENTOR  
*Alvin L. Breen*

BY C. H. Mortenson

ATTORNEY

# United States Patent Office

2,931,091

Patented Apr. 5, 1960

1

2,931,091

## CRIMPED TEXTILE FILAMENT

Alvin L. Breen, West Chester, Pa., assignor to E. I. du Pont de Nemours and Company, Wilmington, Del., a corporation of Delaware

Application February 26, 1954, Serial No. 412,781

9 Claims. (Cl. 28—82)

This invention relates to synthetic textile fibers and particularly textile fibers possessing a permanent crimp.

Various methods have been proposed and used to produce crimped synthetic filaments. The principles of these crimping methods comprise mechanical treatment of the filaments spun in normal fashion as well as application of specific conditions of spinning or after-treating which bring about differential physical properties over the cross-section of the single filaments.

Newer proposals of producing an improved crimp in synthetic fibers comprise the spinning of two or more different materials together so that they form a unitary filament which contains the components in an eccentric relation over the cross-section of the filaments. When, for instance, two materials are used together which possess substantially different physical properties, for example, different residual shrinkage, a crimp is brought about by the application of a suitable after-treatment to the spun and drawn composite filaments. These crimped filaments may be quite satisfactory as long as only relatively small tensions are applied during their use. However, with the application of higher tensions, the crimped filaments of the prior art do not possess the optimum properties and the highest possible crimp retention. Perhaps this is the reason that none of these composite crimped filaments have been commercially produced and used.

It is, therefore, an object of the present invention to provide crimped two- or multi-component composite filaments which have improved recovery properties and higher crimp retention. It is another object of the invention to produce crimped filaments with improved mechanical properties. It is another object to produce crimped filaments having an application of high tensions, as they occur in practical manufacture of fabrics therefrom, a considerably higher crimp retention than heretofore obtainable. Further objects will appear as the description of the invention proceeds.

The term "tensile recovery" is well known (cf. U.S. 2,604,689, Beste and Hoffman, Textile Research Journal, vol. 20, No. 7, July 1950, page 441, and also Texile Fiber Yarns and Fabrics, by E. R. Kaswell, published by Rheinhold Publishing Corporation in New York City, 1953) and is defined as the extent to which a yarn recovers its original length after being stretched, a stress-strain curve being used to determine tensile recovery under the testing conditions. The determination is usually carried out at a constant rate of elongation. For example, a given sample of yarn may be elongated 5% at a rate of 1% per minute, held 30 seconds at the 5% elongation and then allowed to recover at the same rate which it was extended and the recovered length measured. The tensile recovery (in this instance for 5% elongation)

$$= \frac{\text{elongation recovered}}{\text{total elongation}} \times 100$$

Since the extent of recovery varies with the elongation,

2

the tensile recovery values are given for a stated total elongation.

The objects of this invention are effected by producing a crimped composite filament, in which the component having the higher tensile recovery properties is the component subjected to the higher strain on straightening the crimp by an external force. This component will be called the "load bearing" component in the following description of the invention. The new improved crimped filaments of this invention may be obtained by different methods. One method comprises spinning together two or more synthetic polymeric fiber-forming materials, of which the material having the higher shrinkage after drawing has the lower tensile recovery properties, in such a way that the materials form over the cross-section of the single composite filament two or more distinct zones which extend through the entire length of the filament in eccentric fashion, whereby only one, or part of, or all the components take part in forming the surface of the single composite filament, stretching the composite filament, length stabilizing the component or components with the higher shrinkage by the application of heat or other means to the drawn composite filament while it is kept under tension, which results in crystallization of this polymer without affecting the other component or components substantially, and subjecting the thus treated composite filaments in a substantially tensionless state to a shrinking treatment.

An important characterizing feature of this method 30 of the present invention is the discovery that in composite synthetic crimped filaments wherein the load bearing component has the lower tensile recovery properties, the overall properties and particularly the crimp retention of the filaments can be greatly improved by subjecting the drawn composite filaments prior to the development of crimp to a treatment which results in crystallization and length stabilization of the normally load bearing component and which does not affect or only slightly affects the other component. Any treatment 35 which meets these requirements may be used. Such treatments are, for instance, a taut heat treatment at a temperature high enough and for a time long enough to provide crystallization of the desired polymeric component. The temperatures applied in this heat treatment will generally be higher than the apparent minimum crystallization temperature ( $T_1$ ) of the component which is to be length stabilized. The "apparent minimum crystallization temperature" ( $T_1$ ) is defined as the 40 lowest temperature at which a marked rate of density change, which is known to occur simultaneously with crystallization, takes place within six hours. In other instances, crystallization and length stabilization can preferably be brought about by a treatment of the taut composite fiber with certain polar organic liquids which 45 are latent solvents for the amorphous regions of the component to be stabilized.

In the spinning, the polymers are not appreciably blended together in the melt but are fed separately to a shaped orifice where they are simultaneously extruded. 50 The orifice is, then, adapted to receive the components separately for simultaneous extrusion to form a filament in which each component is substantially localized but is held to the other component in an eccentric relation. The extrusion can be such that the components are localized and held together in a "side-by-side" structure in 55 which both components form part of the surface of the composite. The extrusion may also be such that one component forms a core and the other a sheath to form a composite referred to hereinafter as a "sheath-core" structure. In this structure only the sheath contributes to the surface of the composite. With the spinners described herein, melt spinning leads to composites 60

which are generally smooth and have cross-sections which are substantially round with boundary lines that are regular.

The composite filaments are stretched and the resultant stretched filaments are subjected to the length stabilizing treatment and after that treatment they are given a shrinking treatment while they are in a free-to-shrink state. The crimp in the new crimped filaments of this invention is brought about not only by a differential in shrinkage in the components of the composite but by positioning the components in respect to helical crimps so that the component with the better tensile recovery properties is the load-bearing component.

In the figures:

Figure 1 is a plan view of the spinneret assembly shown in Figure 2;

Figure 2, taken on line 2—2 of Figure 1, is a cross-section of a spinneret of this invention showing the routes of polymer in the formation of sheath-core structures;

Figure 3 is taken on line 3—3 of Figure 2;

Figure 4 is taken on line 4—4 of Figure 2;

Figure 5 is a cut taken on line 5—5 of Figure 2;

Figure 6 is a cross-section of a spinneret of this invention showing the flow of polymer in the formation of side-by-side structures;

Figure 7 is taken on line 7—7 of Figure 6;

Figure 8 shows cross-sections of the sheath-core filaments of this invention; and

Figure 9 shows cross-sections of the side-by-side filaments of this invention.

Figure 10 is a sectional perspective of a fragment of a composite in a crimp form referred to as "alpha crimp";

Fig. 11 is a sectional perspective of a fragment of a composite in a crimp form referred to as "beta crimp"; and

Figure 12 is a diagram of apparatus which can be used in applying a process of this invention in a continuous manner.

Referring first to Figure 2 it can be seen that the top component or filter pack 1 of the spinneret has two chambers 2 and 3. Each is fed a different polymer. The chambers are separated by wall 4 and in the bottom of the top portion are a plurality of holes 5 cooperating with outlets below. The chamber 3 and the holes 5 therein cooperate with the grooves or recesses 6 and 23 in the center portion of adapter 7 and feed the polymer melt to the vertical holes 8 or tubes 31. These tubes 31 extend downwardly into the orifices 9 contained in the bottom portion or spinneret face 10. The chamber 2 permits the feeding of polymer downwardly through holes 5 which cooperate with holes 11 in center portion 7 to permit the flow of polymer to grooves or recesses 12 and 29 in the bottom portion 10. The plan views of the top, center and bottom portions may be seen in Figures 1, 3 and 4, respectively. As shown, gaskets 25 are provided for sealing purposes, the assembly being held together by means of bolts or by pressure.

As shown in Figure 2 and in an enlarged manner in Figure 5, polymer 13 coming to the holes 8 or tubes 31 from the chamber 3 constitutes the core feed. As this polymer leaves tube 31 which is surrounded by the melt 14 of polymer coming from chamber 2 and constituting the sheath, bonding occurs so that in the tapered section 30 of orifice 9, polymers 13 and 14 are being extruded simultaneously with polymer 14 completely surrounding the polymer 13. It is to be noted that tube 31 is eccentrically located in the orifice 9. This is done purposely to get the eccentric relation of the polymers, for the more pronounced the eccentricity, the better are the crimp results. As can be seen in Figure 8, the filaments thus produced by melt spinning have substantially round, smooth surfaces. Even the core is substantially round and smooth and in all cases the core does not break through the surface. That is, even in such a filament as 15 there is polymer 14 surrounding the core even though the core comes very close to the outer edge at one place.

In the production of eccentric composite filaments such as sheath-core structures, one uses a material 13 and a material 14 which are so related that material 13 has the better tensile recovery properties. If material 14 has a

higher shrinkage than material 13, the crimped structure shown in Figure 10 wherein the material 14 is located on the inside of the helical coil is obtained. This type of crimp in which the material 14 having the lower tensile recovery properties is located on the inside of the coil 10 is referred to herein as "alpha crimp." Since the material on the inside of the helical coil is the load-bearing constituent of the composite, it is desired to have that material be the material having the better recovery properties. By the process of this invention, it is possible to produce such crimped filaments as are shown in Figure 11. In this figure, material 13 is on the inside of the helical coil and has the better tensile recovery properties. This type of crimp shown in Figure 11 is referred to herein as "beta crimp." As mentioned above, one method of this invention

for producing the desired beta crimp involves the conversion of the alpha crimp type to the beta crimp type. This is referred to herein as "reverse crimp"; in this reversal the material 13 has been converted so that it is now the material having the higher shrinkage while retaining its better tensile recovery properties. As will appear hereinafter, it is also possible by the selection of polymeric materials, heretofore not used, to produce the desired beta crimp without applying the length stabilizing step described above to reverse the alpha crimp.

30 A relatively low tension applied to the crimped filament results in extension of the coils and finally in straightening of the coils because of the very low crimp modulus. Tensions which are higher than the crimp modulus will extend the straightened composite filament 35 whereby the "shorter" component which forms the inside of the coil bears a relatively greater part of the total load applied. It follows therefrom that a relatively higher strain is applied to the load-bearing component than to the coating component in a tensioned crimped 40 composite filament. When the load-bearing component has the lower tensile recovery properties, which is the case with the combinations of synthetic high polymers proposed herebefore for the preparation of crimped composite filaments, the degree and tightness of the crimp will be reduced after application of relatively high loads, 45 because the load-bearing component does not recover as much as its counterpart. The new composite crimped filaments of this invention do not have this disadvantage because the material with the better tensile recovery properties has been made to be the load-bearing component.

50 It is evident from the foregoing that it is of great importance for evaluating crimped composite filaments to have a reliable method for measuring the crimp retention. A commonly used method is described e.g. in U.S. 2,287,099. In this test, relatively low loads, equivalent to 0.03 g./denier are applied to the crimped filaments while immersing them for 30 seconds into water of 60° C. These tensions are much lower than the 55 strain usually imposed on the single filaments in normal use of textile products containing these filaments. Therefore, a more stringent test has been developed, which simulates more the actual conditions encountered in practical use of the crimped filaments.

60 The crimped yarn or filaments are formed into a skein the length of which is measured without applying any tension (a, in centimeters). The skein is then loaded with a weight corresponding to 0.01 g./denier and the straightened length of the skein is measured (b, in centimeters). The skein is then loaded for 30 seconds with a weight corresponding to 1.0 g./denier. The filaments are allowed to recover, after removal of the load, for 30 seconds and the length of the skein is again measured 65 (c, in centimeters).

The crimp permanence is calculated by the following equation:

$$\text{Percent crimp permanence} = 100 \frac{\left(\frac{b}{c} - 1\right)}{\left(\frac{b}{a} - 1\right)}$$

In the examples parts and percentages are by weight.

*Example I*

Poly(ethylene terephthalate) flakes having an intrinsic viscosity of 0.67 in a solvent mixture of 58.8 parts by weight phenol and 41.2% by weight of trichlorophenol and poly(hexamethylene adipamide) flakes having an intrinsic viscosity of 1.02 in m-cresol are melted separately and extruded at 285° C. through a multi-hole spinneret assembly shown in Figure 2. The extruded filament is air quenched. The polyester melt is extruded through the inner tube of the spinneret and the polyamide through the outer space surrounding the tubes, thus forming a sheath-core filament. Figure 8 shows a cross-section of a bundle of the eccentric sheath-core filaments thus obtained. This drawing, based on a microphotograph, shows clearly the eccentric position of the polyester cores in the polyamide sheaths over the cross-section of the single filaments forming the fiber bundle.

The eccentric sheath-core filaments are attenuated by pulling them as they are spun away from the spinneret holes with a speed which is about 100 times as high as the speed of the extruded melt. After spinning and cooling, they are drawn over a pin at room temperature (20° C.) to 3.3 times their original length. About 100 yards of the stretched filaments were tightly wound on a bobbin, and the bobbin was heated for 30 minutes in an electric oven, the temperature of which was 115° C. The cooled filaments were then unwound from the bobbin and showed upon inspection no distinct crimp. However, they possess a potential crimp which can be developed immediately after the heat treatment or at any time after the fiber is processed into woven textile materials or into knitted goods or after cutting the fibers into staple lengths.

*Example II*

A part of the continuous filament of Example I containing the potential crimp was skeined and hung in boiling water for one minute without applying any tension to the filaments. A very tight helical crimp developed instantly. The filaments contained on an average 50 crimps per inch. Microscopic inspection of the filaments showed that the core of poly(ethylene terephthalate) was positioned in the outer portion of the single coil and the thicker parts of the polyamide skin were situated on the inside of the single coil. Therefore, the filaments contained the "beta crimp."

*Example III*

Part of the eccentric sheath-core composite filament yarn of Example I was plied and twisted to a yarn containing 56 filaments with a total denier of 180. The twist was 0.5 turn per inch. This yarn was knit into tubing which when flattened to double thickness measured 3 1/8" wide. A piece of this tubing 12 inches long was placed in boiling water containing 0.5% "Duponol" for 30 seconds. The fabric was then rinsed, centrifuged and dried in the open air. The dry fabric was found to measure 3 1/8" wide and 5 1/8" long. The bulk and covering power of the fabric were correspondingly increased. Moderate tension caused stretching of the fabric beyond the original dimensions but the shrunken form returned almost completely upon release of such tensions. This good shape retention of the boiled-off knit fabric is attributed to the good crimp retention of the crimped fibers composing the fabric.

If the spun and drawn filaments of Example I are

given the shrinkage treatment of Examples II or III without applying first the length stabilization treatment of Example I, highly crimped filaments are obtained. However, microscopic inspection of the cross-section of these crimped filaments shows that the cores consisting of the polyester are positioned on the inner portion of the coils and the thicker portions of the polyamide skin are on the outside of the coils. These fibers therefore possess the "alpha crimp" and do not possess the crimp retention of the "beta" type of this invention.

*Example IV*

Poly(ethylene terephthalate) flakes having an intrinsic viscosity of 0.67 in a solvent mixture comprising 58.8 parts by weight phenol and 41.2 parts by weight trichlorophenol and polyethylene, having an inherent viscosity (0.5% concentration) of 0.88 in tetralin measured at 125° C., were melted separately and extruded at 296° C. through a spinneret as shown in Figure 2. The polyethylene melt was extruded through the inner tube of the spinneret and the polyester through the outer space surrounding the tubes, thus forming a sheath-core filament.

After spinning and winding, the quenched sheath-core filaments were passed through a water bath at 30° C. to a roll heated to 65° C. and then to an unheated roll rotating at a higher speed whereby the yarn was stretched 2.6 times its original length.

A part of this continuous filament yarn was skeined and hung in boiling water for 1 minute without applying any tension to the filaments, whereupon the yarn crimped spontaneously. Microscopic examination of the crimped filaments showed that the heavy part of the polyester skin was situated on the inside of the single filament coil, which corresponds to the "alpha crimp" described above. These "alpha crimped" filaments showed a crimp retentivity of less than 25% when measured according to the new method described above.

Another portion of the freshly spun yarn was wound tightly on a bobbin and immersed in acetone at room temperature for one minute. This yarn was then skeined and hung in boiling water, tension free, for one minute. Crimp developed readily. Crimp retentivity was found to be higher than 90% when measured according to the new method described above. Microscopic inspection of the crimped filaments showed that the crimp was the beta type.

In the foregoing examples the filaments were spun through the spinneret shown in Figure 2 which was found to be especially suited and economical to be used for obtaining a random eccentric sheath-core structure in the single filaments. However, the invention is not limited to the application of this specific spinneret. Any other form of a spinneret which permits production of a composite filament which contains at least two components in an eccentric relationship over the full length of the filament can be used. There are no restrictions with respect to which component forms the core and which component forms the sheath in the sheath-core structures of this invention. Though it is generally preferred to choose the component with the higher tensile recovery properties to form the sheath, other considerations like solubility, spinning technique, appearance and hand, and physical properties may make the reverse order desirable. The invention is further not limited to the eccentric sheath-core filaments. Any other form of a composite filament which contains the components in an eccentric relationship over the cross-section of the single filament may be utilized instead of the sheath-core structure shown in the examples. So for instance, the components can also be spun in the so-called "side-by-side" relationship wherein the components are combined at only part of their surface and both components take part of the surface of the composite filament. However, the "sheath-core" structures are preferred in this invention because

the problem of coherence, which exists with many polymer combinations, particularly on drawing the "side-by-side" structures, in practically eliminated in sheath-core structures. The latter structures therefore permit a much wider application of this principle. Other embodiments include composite filaments which are composed of more than two components. Filaments have been produced in the above examples which consist of about equal parts of the two components. However, sometimes it might be preferred to use a relatively higher amount of one component and a correspondingly lower amount of the other component. Good results can usually be obtained with compositions of at least 20% by weight of one component and 80% by weight of the counterpart up to a ratio of 50% by weight of both components. Those composite filaments containing about equal portions of both components are preferred because of the higher tightness and permanence of the crimp achieved.

Sometimes it might be desirable to spin a bundle of filaments which comprises composite filaments containing the components in various ratios through one and the same spinneret. An example is a bundle of two-component composite filaments which comprises filaments consisting of 20% by weight of the load-bearing component and 80% by weight of the other, a 30%/70% ratio, a 40%/60% ratio and a 50%/50% ratio, respectively. Such filament bundles containing composite filaments with various ratios of components can very conveniently be produced by utilizing the spinneret which is shown in Figures 6 and 7. The spinneret shown is composed of two parts. In the upper portion 16 are two chambers 17 and 18 cooperating with holes 19 in the bottom plate of the top portion. These holes permit the feeding of polymer to grooves or recesses 20 in the bottom portion 21 of the spinneret. The polymer coming from hole 19 goes into the recess 22 immediately below it and is fed to a plurality of recesses 20. Each recess contains and cooperates with a spinneret hole 24. In each spinneret, provision is made for a gasket 25 and conventional means, as by bolting or pressure, can be used to hold the various spinneret elements in place during operation.

However, in the spinneret shown by Figures 6 and 7 there is no tube located in the spinneret orifices 24 such as are in the spinneret orifices 9. Thus, in this modification polymer coming from chamber 17 and the other polymer coming from chamber 18 meet at the orifices 24 and are extruded simultaneously to form side-by-side structures. Cross-sections of such structures are shown in Figure 9, these structures being designated by reference number 26, the parts being 27 and 28.

The spinning, drawing, and length stabilization of the load-bearing component in the composite filament and the after-treatment for bringing about the crimp were described in the foregoing as a discontinuous procedure wherein each treatment was carried out as a separate processing step. The same outstanding results however can be achieved in a fully continuous process. An apparatus especially useful for the continuous procedure is shown in the schematic drawing of Figure 12.

The apparatus comprises a draw pin 32 at which the stretching occurs, a heating medium 33 such as a hot metallic surface, and a draw roll 34. The following Example V is representative of a continuous process for producing the composite filaments having the reversed permanent "beta crimp."

#### Example V

Following the procedure described in Example I, composite sheath-core poly(ethylene terephthalate)-poly(hexamethylene adipamide) filaments are extruded through a spinneret like that shown in Figure 2 having 34 holes. The filaments 35 are attenuated by drawing them from the spinneret at approximately 500 times the

speed with which the polymer leaves the spinneret holes. The bundle of filaments is, after cooling, continually drawn over a draw pin 32 which is heated to 85° C. On its path to the draw roll the filament bundle is led over a hot plate 33 which is heated to 140° C. The total draw imposed on the yarn is 3.56. The filaments, the thickness of which corresponds to approximately 2 deniers, are substantially uncrimped but they possess the potential crimp. Subsequent tensionless treatment in 10 boiling water by short immersion developed readily a tight helical crimp. The crimped filaments have on an average approximately 60 crimps per inch and a crimp elongation of 170% and a crimp retention of 90% when measured according to the above-described test with the 15 application of a load of 1 g./denier for 30 seconds. Microscopic inspection of the crimped filaments showed that the filaments have the beta-type crimp wherein the thicker portions of the polyamide skin form the inside of the single coils.

20 Similar composite filaments produced according to the foregoing method however omitting the length stabilization on the hot plate had a crimp elongation of only 70% and a crimp retention of only 40% when measured by the test used above.

25 Suitable components for producing the permanently crimpable composite fibers by the process which includes the length stabilizing step can be found in all groups of synthetic fiber-forming materials. Because of their commercial availability, ease of processing and excellent 30 properties, the condensation polymers, e.g., polyamides, polysulfonamides and polyesters and particularly those which can readily be melt spun are preferred for application in this method. Suitable polymers can be found for instance among the fiber-forming polyamides and polyesters which are described e.g. in U.S. 2,071,250, U.S. 2,071,253, U.S. 2,130,523, 2,465,319, U.S. 2,130,948, U.S. 2,190,770 and in other places. A preferred group of polyamides comprises such polymers as poly(hexamethylene adipamide), poly(hexamethylene sebacamide), 35 poly(epsilon-caproamide) and the copolymers thereof. Among the polyesters may be mentioned, besides poly(ethylene terephthalate), which is preferred for most applications, the corresponding copolymers containing small amounts of sebadic acid or adipic acid as well as the 40 polyesters containing recurring units derived from glycols with more than two carbons in the chain.

45 Fiber-forming polysulfonamides can be produced by reacting at an interface between two immiscible phases organic sulfonic acid halides, e.g. dichlorides, which form 50 or are contained in one phase, with primary or secondary organic diamines which form or are contained in the other phase, whereby preferably one of the phases is dispersed in the other while the reaction takes place. Such a method is described, for instance, in U.S. Patent 2,667,468.

55 Another group of condensation polymers which can be used in this invention, comprises the polymers which contain sulfonamide groups as well as carbonamide groups. These polymers are conveniently produced by 60 the same method as described above, however, substituting the disulfonic acid halides by the corresponding organic monocarboxylic, sulfonic acid dihalides.

65 The above-described interfacial polymerization methods may also be used for producing the polyamides, when organic dicarboxylic acid halides are used instead of the sulfonic acid halides. When dicarboxylic acid halides are reacted with glycols in the above reactions, the fiber-forming polyesters are obtained. Other groups of polymers useful as components in the filaments of the present invention can be found among the polyurethanes or polyureas which may be made either by conventional methods or by the above-described interfacial methods as well as among the polyvinyl compounds including such polymers as polyethylene, polyacrylonitrile, polyvinyl 70 chloride, polyvinylidene chloride, and similar polymers.

It is evident from the foregoing description that the compounds are operative in the method comprising the length stabilization step only when the materials are combined in the composite filaments in such a way that the "normally load-bearing" component which is the component with the higher shrinkage can be length stabilized under conditions which do not substantially reduce the residual shrinkage of the other component so that a differential in shrinkage of at least 5% and preferably 10% or more is achieved. Actually, after the length stabilizing treatment, the "normally load-bearing" component has a lower shrinkage than the other component and reversal of crimp results. The physical properties and particularly those properties as residual shrinkage, tensile recovery, or permanent set by extension among others of the fiber-forming polymers are well known and can easily be determined. Therefore, by comparing the physical property data of the desired components, the operability of any given combination according to the present invention can easily be determined by following the teachings given herein.

The fiber-forming high polymeric materials can be length stabilized by crystallizing the polymer under conditions wherein no shrinkage can occur. In other words the crystallization is effected under conditions of tension which equals the forces developed in the filaments during the treatment. Crystallization or length stabilization respectively of many of the fiber-forming high polymeric materials can therefore be accomplished preferably by a heat treatment of the taut filaments. This is usually applied when the "normally load-bearing" component—in Example I this is the poly(ethylene terephthalate)—has the lower apparent minimum crystallization temperature ( $T_1$ ).  $T_1$  for poly(ethylene terephthalate) is 99° C. The temperature applied should generally be higher than the apparent minimum crystallization temperature of the "normally load-bearing" component which is well known or can easily be determined for each polymer. A convenient method for determining the apparent minimum crystallization temperature ( $T_1$ ) is described e.g. in U.S. 2,578,899. In order to achieve the results of the present invention, namely, length stabilizing one component and not affecting to a substantial extent the residual shrinkage of the other component, a temperature is preferably chosen which is lower than the apparent minimum crystallization temperature of the counterpart. However, depending on the nature of the other component or components in the combination and the length of time of exposing the composite filaments to the taut heat treatment, a higher or lower temperature can be chosen to achieve optimum results and the tightest possible crimp. The temperature range for the taut heat treatment may vary in wide limits and may be up to about 100° C. or more above  $T_1$  of the "normally load-bearing" component. Usually, however, best results are obtained when applying a temperature in the range of 5° C. to 70° C. above  $T_1$  of the "normally load-bearing" component. The lower temperatures in this range are applied when the composite filaments are exposed to the taut heat treatment for longer periods of time, e.g. for 30 to 60 minutes, while the higher temperature range is applied with shorter heat treatments, e.g. of some minutes or seconds or less. The temperature of the heat treatment should in any event, however, be lower than the softening or melting temperature of the lower melting component in the composite filament. For a given combination with a given set of processing conditions, however, the temperature of the taut heat treatment is very critical and usually should be kept in a range of plus or minus 10° to plus or minus 15° of its optimum temperature in order to achieve maximum results. In the continuous process shown in Example V the temperature of 140° C. at the hot plate should be maintained within the limits of approximately plus or minus 10° C. in order to produce a yarn with maximum crimp retention and crimp tight-

ness. If optimum properties are not desired, the temperature of the hot plate could be varied in limits of about plus or minus 15 to 20° C. Even though the temperature of the draw pin is not as critical as the temperature of the hot plate, it should not vary more than approximately 30° C. and preferably 15° C. from the temperature of 85° C. used in the foregoing example. As already pointed out with varying spinning and processing conditions and with different combinations of materials, the optimum temperatures may vary in wide limits.

It is known that not only elevated temperatures bring about crystallization and length stabilization of a given polymer but also other special conditions under which the material is treated. Thus, for instance, the presence of plasticizers has a great effect on the temperatures necessary to achieve crystallization and reduction of residual shrinkage. This can be utilized in the present invention by adding a plasticizer to the "normally load-bearing" component. This can be an organic plasticizer as commonly used in polymer applications which may be subsequently removed. Water may take the function of a plasticizer especially when the two polymers differ in their ability to absorb moisture.

On the other hand, for instance, when poly(hexamethylene adipamide) and poly(ethylene terephthalate) are used in a combination wherein the polyamide forms at least part of the outer skin of the composite filament, it is advantageous to remove most of the moisture from the polyamide before or while applying the taut heating step of this invention. The reverse situation may be true with other combinations. By varying these conditions, as well as the lengths of time of the heat treatment and/or the temperature of the treatment, the tightness of crimp and crimp permanence can be varied. In order to obtain a crimp as tight as possible, optimum conditions for the stabilizing treatment are generally observed.

With some combinations of high polymeric materials it is not possible to avoid fully the reduction of residual shrinkage of the co-acting compound or compounds in the composite filaments when the length stabilization is brought about by heating to a temperature higher than the apparent minimum crystallization temperature of the normally load-bearing component. This is true, for instance, when the "normally load-bearing" component has a higher apparent crystallization temperature than its counterpart. In these instances and also for other reasons, sometimes other methods might be preferred for crystallizing or length stabilizing the normally load-bearing component. A very convenient method comprises the exposure of the composite filament, while in taut condition, to the action of certain polar organic liquids which are latent solvents for the amorphous regions of the load-bearing component and which therefore promote crystallization of the normally load-bearing component but do not affect the other component or components substantially. A suitable liquid will be chosen depending on the specific combination of polymeric materials. In a combination of polyethylene and poly(ethylene terephthalate), for instance, acetone has proven to be an excellent material to promote crystallization of the poly(ethylene terephthalate). Other suitable polar liquids are, for instance, chloroform, methylene chloride, tetrachloroethane, phenol, m-cresol among others. In those liquids having too great swelling action, dilution with water or other less active liquids may be necessary. Temperatures and other conditions of the liquid treatment may be varied in wide limits with various combinations of polymers to achieve every desired result with respect to the tightness, permanence and appearance of the "beta crimped" filaments. Example IV above shows the preparation of a composite filament from polyethylene and poly(ethylene terephthalate), using a liquid treatment for length stabilization.

In addition to the methods described above involving length stabilization, there is another method for producing

the new composite crimped filaments of this invention. This method does not require the length stabilizing step. This method comprises spinning together two or more synthetic polymeric fiber-forming materials, of which the material having the higher shrinkage after drawing also has the higher tensile recovery properties. The spinning is done as before so that the materials form over the cross-section of the single composite filament two or more distinct zones which extend through the entire length of the filament in eccentric fashion, whereby only one or part of, or all the components take part in forming the surface of the single filament, stretching the composite filament, and subjecting the drawn composite filaments, in substantially tensionless state to a shrinking treatment. In this method, synthetic high polymers forming the load-bearing component should have a residual shrinkage of at least 10% and preferably more than 15% after drawing them at least to twice the original length and a tensile recovery of at least 90% at 50% of the elongation-at-break combined with a high extensibility, corresponding to at least 10% and preferably 20% elongation-at-break. Depending on the shrinkage characteristics of the co-acting component, even higher limits of these values may be necessary to produce a differential in shrinkage between the two materials of at least 10%.

Synthetic, fiber-forming polymeric materials having the high tensile residual shrinkage and high recovery properties combined with the high extensibility required by this process, which does not require the length stabilization step, are generally not found among the polymers commonly used for producing fibers. However, a limited number of newer polymers which are produced at preferably moderate temperatures, e.g. according to the above-mentioned interfacial polymerization methods, fulfil these requirements in an ideal way. Such polymers are described for instance in copending patent applications Serial No. 345,728, filed March 30, 1953, now Patent No. 2,731,446 to Wittbecker and Serial No. 359,975, filed June 5, 1953, and now abandoned. As co-acting components can be chosen any fiber-forming synthetic polymer which can be spun with the "load-bearing" component and which has a residual shrinkage at least 5% and preferably 10% lower than the "load-bearing" component. These physical properties can easily be determined by the commonly used and generally known testing methods.

The conditions applied for drawing the spun multi-component filaments of this invention may vary in wide limits. Instead of using a pin as mentioned in Example I, other convenient means for drawing the filaments may be applied, for instance, rolls being driven at different speeds. Also, the temperatures at which the filaments are drawn may vary in wide limits and depend mostly upon the properties of the single materials forming the composite filament and of the final desired results. As is the case in the production of conventional unitary filaments, the preferred drawing temperatures for the composite filaments of this invention may vary between room temperature or slightly elevated temperatures and temperatures of about 100° C. up to relatively high temperatures which may in some cases be as high as about 70° C. below the melting point of the lower melting material. Since in the present invention combinations of at least two different materials are employed, the specific drawing characteristic of each material used should be considered in order to obtain best results. In general, it is of advantage to use drawing temperatures which are lower than the apparent minimum crystallization temperature ( $T_i$ ) of the "normally load-bearing" component. This latter limitation of the drawing temperature may become of particular importance in the method which employs the length stabilization step.

The composite filaments have been produced in the examples by the melt spinning technique. Naturally,

also any other spinning method like "plasticized melt" spinning, dry spinning, wet spinning, can be employed successfully. In some instances, particularly when the melting behavior or the solubility of the components in a combination would not permit spinning the components by similar methods, a combination of dissimilar methods is indicated. Thus, for instance, one component, preferably the component forming the sheath can be spun as a solution in a high boiling solvent or as a plasticized melt, while the core-forming component is extruded as the molten polymer. Similar combinations of spinning methods can be used for spinning "side-by-side" structures. In these instances, the solvents or plasticizers may be wholly or partially removed subsequently, preferably by washing them out by the help of low boiling solvents.

In the method involving length stabilization, as shown in Example I, the composite filaments are substantially uncrimped after the application of the length stabilization treatment but contain, however, a "potential crimp." The crimp can be developed in these filaments very readily by a suitable after-treatment. The filaments containing the "potential crimp" can be processed as any ordinary uncrimped continuous filaments or staple fibers to worsted or knitted goods. The crimp can then be imposed on the filaments at any time by a suitable relaxing or shrinkage treatment. This shrinkage treatment was performed in the foregoing examples by exposing the composite filament containing the potential crimp to boiling or hot water. Good results, however, may also be obtained, for instance, by the application of moist heat or steam. Which of these after-treatments for bringing about the crimp are chosen depends mostly on the properties of the components forming the composite filaments and on the final properties which are desired in the crimped filaments. In general, the temperature applied in the crimping procedure should be higher than the apparent second-order transition temperatures ( $T_g$ ) of the polymers forming the composite filament in order to achieve the favorable results of the invention. The apparent second-order transition temperature ( $T_g$ ) of a polymer is defined as the temperature at which a discontinuity occurs in the curve of a first derivative thermodynamic quantity with temperature. A convenient method for measuring this temperature is shown in U.S. Patent No. 2,578,899. Since water acts as a plasticizer in many polymers, thus lowering the apparent second-order transition temperature ( $T_g$ ), this should also be considered in measuring  $T_g$  and in selecting the appropriate crimping method and temperature. Other factors influencing the optimum condition for crimping the composite filaments of this invention are, for instance, the spinning, drawing and length stabilizing conditions used and also other factors, for instance, whether the composite filament is processed as continuous filament or as staple or as a woven or knitted textile fabric. Therefore, by varying the after-treating conditions for bringing about the crimp, also the properties and appearance of the crimped filaments can be varied to a great extent in any desired way.

In summary, polymers which are useful as the load-bearing component in the fibers of this invention to produce useful textile materials may be determined by subjecting a filament from the polymer to the processing steps of this invention in the absence of other components and testing certain properties of the resultant filament. Such a filament should have (1) a minimum initial modulus of at least 5.0 grams per denier, (2) a shrinkage of at least 7%, (3) a permanent set at an extension that corresponds to 50% of its elongation-at-break of below 10% and (4) the elongation-at-break should be higher than 15%.

In general, the composite filaments are drawn from about 2 times to about 8 times their original lengths. Prior to drawing the filaments are attenuated; that is, they are slenderized by pulling the freshly extruded filaments away from the orifice at a rate faster than the

extrusion rate. The drawing or orientation step is in addition to attenuation, but also has a slenderizing effect. The extent of drawing will, of course, also depend somewhat upon the nature of the particular polymers used in the composite filament and upon the type of eccentric relationship between those polymers in the composite filament.

In the hot relaxing treatment of this invention used to develop the potential crimp, the medium may be any inert atmosphere capable of being heated to a temperature of about 100° C. Thus, the filaments may be heated in air, nitrogen, hot or boiling water, carbon dioxide or any gaseous or liquid media inert to the polymers in the composite filaments. The temperature used is generally in the neighborhood of 100° C., but it may be lower or higher. For example, any temperature above about 50° C., but below the melting point of the lowest melting polymeric constituent in the composite fiber, may be used. Generally, a temperature in the range of about 50° C. to about 150° C. is used with convenience.

The length of time that the composite filaments are subjected to the hot, relaxing treatment is not critical, because the crimp develops immediately and spontaneously. Thus, the time may be very short, as, for example, a matter of seconds, although it may be desired in some cases to continue the length of treatment for a longer period of time such as 30 minutes, or even for several hours.

Further, the spinnerets described herein may be simplified in certain respects. To illustrate, the tube 31 in the spinneret shown in Figure 2 may be dispensed with, for hole 8 in the adapter is eccentrically located above and in respect to orifice 9, and the jetting of polymer 13 into the melt of polymer 14 and the polymer flow thereafter leads to a sheath-core structure. Also, the provision of recesses 23 of relatively large area in conjunction with channels 6 of smaller area, as shown in the spinneret assembly given in Figure 2, results in the formation of ridges between the channels. These ridges can be removed both in the adapter or spinneret plate. That is, one very large recess is provided, the orifices being appropriately placed, and the polymer fed under pressure flows to the various orifices.

The crimped two-component filaments of this invention show a tight permanent crimp. The crimp obtainable in this invention corresponds usually to more than 10 crimps per inch and up to 300 crimps per inch. The crimp permanence is 50% up to 100% when measured and calculated by the test described above, and those composite filaments having a crimp permanence of about 80% or more are preferred.

It is well known that, in many applications of the continuous or staple-length crimped filaments in textile materials, sometimes relatively high tensions are applied to the fabrics and thus to the single filaments in daily use of these materials. Therefore, high crimp retention, also under high tensions, which is necessary for dimensional stability of the worsted or knitted goods from these crimped filaments is very important for practical application of the crimped filaments.

The characteristic of the new crimped filaments containing the "beta crimp" to retain the original high crimp also after the application of high tensions or high loads to the filaments makes them especially useful for many textile applications where bulky highly crimped filaments are desired and where high crimp retention under high stress is of great importance. This applies also to the crimped filaments which are cut to staple length and which are usually spun into yarns and processed according to known textile processing methods to knitted or woven goods. The new staple filaments of this invention can be crimped before they are further processed or in any state of processing, for instance, after they are spun into yarns or after the woven or knitted goods

are made from these yarns. Another important application comprises the processing of the continuous filaments into bulky fabrics which again can be carried out with the continuous filaments in the crimped or uncrimped state. In the latter case, the crimp can be developed after weaving or knitting the yarns obtained therefrom or in any stage of the processing. Very interesting applications of the continuous yarns are, for instance, the preparation of worsted fabrics which may be woven from the uncrimped yarns containing the potential crimp and which are crimped after weaving and finishing. These worsted fabrics have an appearance and hand very similar to those obtained from staple yarns. However, they do not possess the disadvantages in processing and use of these fabrics. Another very important application of the fibers of this invention comprises the use in carpets and other heavy textile goods where again the fibers containing the potential crimp can be knitted or woven and the crimp is developed in the finished goods.

Any departure from the above description which conforms to the present invention is intended to be included within the scope of the claims.

I claim:

- 25 1. A helically crimped filament comprising at least two different, synthetic polymers one of which constitutes the load-bearing component in said filament, the said polymers having different recovery properties and being contained in said filament as substantially separate components held together in eccentric relation to each other, the load-bearing polymeric component of said filament being located at the inner portion of the helical coils and being the polymer having the better tensile recovery properties.
- 30 2. A filament in accordance with claim 1 wherein said relation is a sheath-core relation.
- 35 3. A filament in accordance with claim 1 wherein said relation is a side-by-side relation.
- 40 4. A filament in accordance with claim 1 wherein one of said polymers is a polyamide.
- 45 5. A filament in accordance with claim 1 wherein one of said polymers is a polyester.
- 50 6. A filament in accordance with claim 1 wherein one of the said polymers is a poly(ethylene terephthalate).
- 55 7. A filament in accordance with claim 2 wherein the load-bearing component is a polyamide and said polyamide constitutes the sheath.
- 60 8. A helically crimped filament made from at least two synthetic polymers differing in recovery properties, one of which polymers being the load-bearing constituent in said filament, said filament comprising a polyamide and a polyester having different recovery properties and contained in said filament as substantially separate components held together in eccentric relation to each other, the said polyamide being the load-bearing constituent appearing at the inner portion of the helical coil and being the polymer having the better tensile recovery properties.
- 65 9. A filament possessing potential crimp comprising at least two different, synthetic polymers one of which constitutes the load-bearing component in said filament, the said polymers having different recovery properties and being contained in said filament as substantially separate components held together in eccentric relation to each other, said filament being capable of developing a permanent helical crimp wherein the load-bearing component appears at the inner portion of the helical coil and has the better tensile recovery properties.

References Cited in the file of this patent

UNITED STATES PATENTS

- 2,238,694 Graves ----- Apr. 15, 1941  
2,386,173 Kulp et al. ----- Oct. 2, 1945

(Other references on following page)

15

## UNITED STATES PATENTS

|           |               |                |           |
|-----------|---------------|----------------|-----------|
| 2,428,046 | Sisson        | Sept. 30, 1947 | 2,674,025 |
| 2,439,813 | Kulp et al.   | Apr. 20, 1948  | 2,716,049 |
| 2,439,814 | Sisson        | Apr. 20, 1948  | 2,737,436 |
| 2,439,815 | Sisson        | Apr. 20, 1948  | 5         |
| 2,440,761 | Sisson et al. | May 4, 1948    | 514,638   |
| 2,612,679 | Ladisch       | Oct. 7, 1952   |           |

16

|         |               |
|---------|---------------|
| Ladisch | Apr. 6, 1954  |
| Latour  | Aug. 23, 1955 |
| Boeuf   | Mar. 6, 1956  |

## FOREIGN PATENTS

|               |               |
|---------------|---------------|
| Great Britain | Nov. 14, 1939 |
|---------------|---------------|